

# United States Patent Office.

EDWARD J. HILL, OF MILWAUKEE, WISCONSIN.

*Letters Patent No. 72,637, dated December 24, 1867; antedated December 10, 1867.*

## IMPROVEMENT IN THE MANUFACTURE OF MATCHES.

The Schedule referred to in these Letters Patent and making part of the same.

### TO WHOM IT MAY CONCERN:

Be it known that I, EDWARD J. HILL, of the city and county of Milwaukee, and State of Wisconsin, have invented a new and improved Mode of Manufacturing Friction or Percussion-Matches, Tapers, and Cigar, Gas, or Lamp-Lighters; and I do hereby declare that the following is a full and exact description thereof, reference being had to the accompanying specimens, &c., and to the letters of reference marked thereon, making a part of this specification.

The nature of my invention consists in the application of a principle or property or quality of the parts, masses, or compounds used generally in the manufacture of friction or percussion-matches, tapers, cigar, gas, or lamp-lighters, of which property or quality I claim to be the discoverer, namely, the property or quality of being cut (particularly by shears, or cutting-machines working on the principle of the shears, or in any other way, without producing friction or percussion,) after such pastes, masses, or compounds have become dry and hard, so that when placed on thin sheets of wood, paper, cloth, webs of yarn, twine, thread, or any other suitable substance, or otherwise, any such material may be marked off with the paste-like ink, or strips thereof, of proper and convenient width, if desirable, may be dipped and dried, and then cut with much greater facility and less labor than in any of the known modes now in use; in other words, a large match may be made, say one or more yards long, and the same may be divided indefinitely, each piece becoming a perfect match; the same as to tapers and lighters, to wood, and to all other substances used in their construction, as well as in the original use of wood, paper, twine, cloth, and other suitable material, in such manner for friction or percussion-matches, tapers, and cigar, gas, and lamp-lighters; and also in the original use of twine, yarn, or thread, for friction or percussion-matches; and also in the peculiar manner of putting up or packing friction or percussion-matches, tapers, cigar, gas, and lamp-lighters, so that each, when drawn from its original wrapper or case, will be ignited for use, making the wrapper or case and match, taper, or lighter, inseparable, except for use, unless it be desired to separate them, should recasing demand, and in protecting the pasted ends of matches, tapers, and lighters, as herein specified.

To enable others skilled in the art to make and use my invention, I will proceed to describe its construction and operation.

I make my matches, tapers, cigar, gas, or lamp-lighters, in any of the known forms, but prefer flat or square splints, strips, or slips of any suitable material. I reduce the material to thin sheets, which I cut into strips of the length of two matches or tapers or lighters, which strips may be dipped in any of the known substances now generally used, to render the same highly inflammable, then dried, and dipped in almost any of the compounds known or used, for the purpose of producing ignition, either by friction or percussion, but I prefer the following compound: four parts phosphorus, ten parts nitrate of potash, six parts of fine glue, five parts of red lead, and one part fine smalt; or for tapers and paper matches, the following compound or formula: gum-arabic, sixteen parts; phosphorus, nine parts; nitrate of potash, fourteen parts; manganese, sixteen parts. Mix so as to form a perfectly homogeneous mass. If desirable, the quantity of phosphorus may be diminished to five parts.

I convert the glue, with a little water, by a gentle heat, into a smooth jelly, put it into a slightly-warm porcelain mortar, to liquefy, rub the phosphorus down through this gelatine, at a temperature of about  $140^{\circ}$  to  $150^{\circ}$  Fahrenheit, add the nitre, then the red powder, and lastly the smalt. I dip the edges of the strips, which should be thoroughly dry, in this mass or paste, from one-sixteenth to one-eighth of an inch deep. If the strips be thin, one-fourth of an inch deep will be better. Then I thoroughly dry the same for from four to six hours; then varnish the dipped portion, by dipping the same in thin varnish prepared from almost any of the gum resins in the usual manner, but for tapers and paper matches, I prefer the double tincture of benzoin, or its equivalent. The effect of the varnish is to protect the paste, rendering it safe and better to handle, giving inflammability to the body of the match, without the use of sulphur or wax, or other substances, and preserving the same from absorbing moisture, and protecting it from accident. These strips may then be cut with the shears, or machines acting on the principle of the shears, or in any other way, so as not to produce percussion or friction, into any convenient or desirable size for use, and put up in any of the known forms now in use; but I prefer to cut the same, leaving a margin, so as to handle them in cards, and to put them up in my friction-

wrappers or cases, folding them into paper, cloth, sand-paper, or prepared paper roughened, or any other suitable material, protecting the pasted ends in the folds of the sand-paper, as in the samples herewith accompanying this specification.

I construct matches of paper or twine, also, by cutting the paper in strips of suitable width, say from one-sixteenth to one-fourth inch in width, and then placing these strips or twine in a frame, making a web of at least one hundred strips or strands, and then apply the paste by strips of wood or frames or brushes, drawn across the web at convenient distances. I then cut and fold as before. When paper is used, by making or pasting the sheets or strips crosswise, and cutting the same in narrow strips, from one-sixteenth to one-fourth inch wide (or with twine or yarn or thread, by not cutting,) I get continuous bands, ribbons, or strings of matches, attached together longitudinally, which I put up for use in boxes, and in friction or percussion-cases, in manner similar to the samples herewith sent. A pin, or point of a knife or needle, or other sharp-pointed instrument, scratched across the paste, will produce ignition instantly.

What I claim as my invention, and desire to secure by Letters Patent, is—

1. The discovery of the quality or property of the mass or paste usually employed to produce ignition in matches, tapers, lamp, cigar, or gas-lighters, which permits the same to be cut without friction or percussion, especially when spread in thin sheets of suitable material, after the same has become dry.
2. The use of twine or yarn or thread, or equivalents, in the manufacture of friction or percussion-matches.
3. The peculiar manner of placing the twine, yarn, or thread for dipping, as herein described.
4. The particular combinations to produce the results respectively herein described, or in any other substantially the same, as shown by each of the specimens accompanying this specification.
5. The putting up and packing matches, tapers, and lighters, in friction-wrappers, cases, or holders, or otherwise, so as to unite the match, taper, or lighter, with the case or wrapper, making the same go hand in hand with each other, in the various combinations herewith presented, and all permutations thereof.
6. The application of varnish after dipping, as herein described, or otherwise.
7. I claim paper for matches, as herein specified, in the combinations set forth.
8. The protection of the pasted ends of the matches, tapers, or lighters, in manner and form, by folded paper or other suitable material, as in this application described.

EDWARD J. HILL.

Witnesses:

J. S. CLARK,  
E. E. HILL.